

## [54] TREATMENT OF FIBRES

[75] Inventors: **Albert John Barber**, Sale; **Derek James Rowland Massey**, Linton, both of England; **James McCartney**, Banbridge, Northern Ireland; **Kenneth Winterbottom**, Whittleford, England

[73] Assignee: **Ciba-Geigy AG**, Basle, Switzerland

[22] Filed: **Apr. 12, 1972**

[21] Appl. No.: **243,470**

## [30] Foreign Application Priority Data

Apr. 19, 1971 Great Britain ..... 9765/71

[52] U.S. Cl. .... **117/138.8 A**, 8/115.6, 117/138.8 B, 117/138.8 F, 117/138.8 N, 117/138.8 UA, 117/138.8 PV, 117/139.5 A

[51] Int. Cl. .... **D06m 15/48**, D06m 15/08

[58] Field of Search ..... 8/115.6, 185; 117/139.5 A, 117/138.8 B, 138.8 F, 138.8 N, 138.8 A

## [56] References Cited

## UNITED STATES PATENTS

|           |         |                |             |
|-----------|---------|----------------|-------------|
| 2,461,920 | 2/1949  | Pratt .....    | 260/828 X   |
| 2,917,410 | 12/1969 | Vitalis.....   | 117/139.5 X |
| 3,476,697 | 11/1969 | Clements ..... | 117/139.5 X |

|           |         |                        |             |
|-----------|---------|------------------------|-------------|
| 3,498,821 | 3/1970  | Hanson .....           | 8/115.6 X   |
| 3,690,942 | 9/1972  | Vandermaas et al. .... | 117/139.5 X |
| 3,703,352 | 11/1972 | Dobinson et al. ....   | 117/141 X   |
| 3,706,527 | 12/1972 | Dobinson et al. ....   | 8/115.6 X   |
| 3,706,528 | 12/1972 | Dobinson et al. ....   | 117/139.4 X |

Primary Examiner—Herbert B. Guynn

Attorney, Agent, or Firm—Joseph G. Kolodny; Edward McC. Roberts; Prabodh I. Almala

## [57] ABSTRACT

Synthetic textile materials, such as polyamides, polyesters, polyacrylonitrile, polyvinyl alcohol, and cellulose triacetate, are treated with an ester containing on average, at least two mercaptan groups per molecule, which is then cured, in order to impart a better handle and improved antisoil properties.

Typically, the ester is prepared by the reaction of

- a compound containing at least two carboxylic acid groups
- a compound containing at least two alcoholic hydroxyl groups and, optionally,
- a compound containing not more than one carboxylic acid group or alcoholic hydroxyl group, especially a monomercaptomonocarboxylic acid or a monomercaptomonohydric alcohol.

10 Claims, No Drawings

## TREATMENT OF FIBRES

This invention relates to a process for modifying synthetic materials in fibrous form, and to materials so treated.

It is well known to treat textiles comprising synthetic fibres with softening agents, such as polyethylene emulsions or adducts of ethylene oxide with phenols or amines, to improve the handle of the textile. These softening agents suffer from the disadvantage of failing to exhaust onto the textile. Since the softening agent is normally applied to a wet fabric just after scouring or dyeing has been carried out, a high concentration of softening agent is required to give the desired uptake, and a high proportion of this softening agent is subsequently removed from the material on washing. The process is therefore wasteful.

It has now been found that, by the use of certain esters containing mercaptan ( $-SH$ ) groups, synthetic fibrous materials having improved properties, in particular textiles having a fuller, softer, and more resilient handle, and improved antisoil properties (including enhanced soil-release, and reduced soil-redeposition) and antistatic properties, can be obtained. These esters may also serve as spinning lubricants and as knitting and weaving oils. It has also been found that, surprisingly, these substances can exhaust onto the fibres and the effects are resistant to washing and dry cleaning.

Accordingly, the present invention provides a process for modifying synthetic fibres which comprises

1. treating the fibres, in the absence of keratinous material, with an ester which contains on average at least two mercaptan groups per molecule and which is obtainable by the reaction of
  - a. a compound containing at least two carboxylic acid groups,
  - b. a compound containing at least two alcoholic hydroxyl groups, and optionally,
  - c. a compound containing not more than one carboxylic acid group or alcoholic hydroxyl group, at least one of (a) and (b), and (c) if used, having one or more mercaptan groups, and
2. curing the ester on the fibres.

The present invention further provides synthetic fibrous materials, free from keratinous materials and bearing thereon an ester as aforesaid, in the cured or still curable state.

Synthetic fibres which may be subjected to the process of the present invention may be in the form of loose fibres, yarns, threads, woven, non-woven and knitted fabrics and garments, woven and tufted carpets, and needle-punched and other mechanically formed fibrous floor covering materials, and are preferably polyamides (nylons), polyesters, polyacrylonitrile, and polyvinyl alcohol. The term "synthetic fibres" is taken herein to include man-made fibres of cellulosic origin in which all three available hydroxyl groups per anhydro-glucosidic unit have been chemically modified, e.g., by acylation, etherification, or cyanoethylation. Thus, cellulose triacetate is regarded, for the purposes of this invention, as a synthetic material.

Mixtures of two or more synthetic fibrous materials, or blends with cellulosic materials, may also be treated, but blends of these materials with keratinous fibres are not included within the scope of the present invention.

Preferred esters for use in the process according to the invention are those esters containing on average not more than six mercaptan groups per molecule, and they usually have an average molecular weight of between 400 and 10,000, but, if desired, esters having an average molecular weight of up to 20,000, or even 40,000 may be used.

Such esters may be those obtainable by the reaction, in any desired sequence, of

- 10 d. a monomercaptomonocarboxylic acid or a monomercaptomonohydric alcohol,
  - e. a compound containing two, but not more than two, alcoholic hydroxyl groups per molecule, and
  - 15 f. a compound containing, per molecule, at least three carboxylic acid groups.
- If desired, components (e) and (f) may be caused to react to form a hydroxyl or carboxyl-terminated ester and this is then esterified with (d).
- 20 Such esters may also be those obtainable by the esterification of
    - g. a monomercaptodicarboxylic acid with
    - h. a compound containing at least two but not more than six alcoholic hydroxyl groups per molecule and, optionally,
    - i. a dicarboxylic acid containing no mercaptan group, or an anhydride of such an acid, or
    - j. a monocarboxylic acid, preferably a monomercaptomonocarboxylic acid, or
    - k. a monohydric alcohol, preferably a monomercaptomonohydric alcohol.
- Similarly, there may be employed esters obtainable by the reaction, in any desired sequence, of
- 30 d. a monomercaptomonocarboxylic acid, or a monomercaptomonohydric alcohol
  - 35 1. a compound containing at least three alcoholic hydroxyl groups per molecule, and
  - m. a compound containing two, but not more than two, carboxylic acid groups per molecule.

As those skilled in the art of making polyesters will appreciate, a carboxylic anhydride may be used in place of the corresponding carboxylic acid while a 1,2-epoxide may be substituted for an alcohol, one epoxide group corresponding to two alcoholic hydroxyl groups.

The esters are prepared in a known manner, preferably by heating the reactants together in the presence of a catalyst such as a strong acid (especially an anion exchange resin, toluene-p-sulphonic acid, or 50 percent sulphuric acid), and of an inert solvent, such as toluene, xylene, trichloroethylene, or perchloroethylene, with which water formed in the reaction can be removed as an azeotrope.

Substances containing at least two carboxylic acid groups, or anhydrides thereof, which may be used as compound (a) include succinic, adipic, phthalic, hexahydrophthalic, sebacic, malic, citric, tricarballylic, pyromellitic, and dimerised or trimerised fatty acids, and their anhydrides (where existing), and thiomalic acid, HOOCCH<sub>2</sub>CH(SH)COOH, otherwise known as mercaptosuccinic acid.

Monomercaptomonocarboxylic acids used as component (d) are usually of formula HOOC-R-SH, where R denotes a divalent organic radical, the indicated HOOC— group being directly bound to a carbon atom of the radical R and the indicated —SH group being directly bound to the same or to a different carbon atom

of the radical R. Preferably they are also of formula HOOC-C<sub>2</sub>H<sub>2r</sub>-SH, where r is a positive integer of from 1 to as high as 18 or even 24. There may be thus be used mercaptoundecylic acid, mercaptostearic acid and especially thioglycollic acid and 2- and 3- mercaptopropionic acid, i.e., r in the above formula is 1 or 2. Mercaptan-containing aromatic acids such as o- and p- mercaptobenzoic acids may also be used.

Monomercaptomonohydric alcohols used as component (d) commonly have the general formula HO-R'-SH, where R' denotes a divalent organic radical, the HO— group and the —SH group being directly bound to carbon atoms of the radical R'. Preferably they are also of formula HO-C<sub>2</sub>H<sub>2t</sub>-SH, where t is a positive integer of from 2 to 18 and especially preferred are those of the foregoing formula where t is 2 or 3, such as 2-mercaptopropano, 1-mercaptopropan-2-ol, and 2-mercaptopropan-1-ol, but substances such as 1-chloro-3-mercaptopropan-2-ol may also be used.

Compounds containing at least three carboxylic acid groups, or anhydrides thereof, which may be used as component (f) include citric acid, tricarballylic acid, pyromellitic acid and trimerised linoleic acid and their anhydrides (where existing).

The monomercaptodicarboxylic acid (g) is usually of formula



where R'' represents a trivalent aliphatic or alicyclic radical, the indicated carboxyl group and mercaptan group being directly linked to a carbon atom or carbon atoms of the group R'', and preferably it is thiomalic acid.

The substances containing at least two alcoholic hydroxyl groups (b,e,h,l) include ethylene glycol, propylene glycol, propane-1,3-diol, butane-1,2-diol, butane-1,3-diol, butane-1,4-diol, hexane-1,6-diol, poly(oxethylene) glycols, poly(oxypropylene) glycols, poly(oxybutylene) glycols, poly(oxy-1,1-dimethylethylene) glycols, poly(epichlorohydrins), glycerol, 1,1,1-trimethylethane, 1,1,1-trimethylolpropane, hexane-1,2,5-triol, hexane-1,2,6-triol, 3-hydroxymethylpentane-2,4-diol, pentaerythritol, mannitol, sorbitol, and adducts of ethylene oxide or propylene oxide with such alcohols, including mixed polyhydric polyethers obtained by treating an initiator containing active hydrogen, such as ethylene glycol, with, say, propylene oxide, and then "tipping" the adduct with a second alkylene oxide, say, ethylene oxide.

Mono-1,2-epoxides which may be used in place of a dihydric alcohol include: ethylene oxide, propylene oxide, butylene oxide, 1,1-dimethylethylene oxide, epichlorohydrin; glycidyl ethers of alcohols (such as n-butyl and iso-octyl glycidyl ethers) or of phenols (such as phenyl and p-tolyl glycidyl ethers), N-glycidyl compounds (such as N-glycidyl-N-methylaniline or N-glycidyl-n-butylamine), and glycidyl esters of carboxylic acids (such as glycidyl acetate).

In place of trihydric and higher alcohols there may be used monoepoxymonohydric alcohols such as glycidol, or a diepoxide such as a diglycidyl ether of an alcohol or a phenol.

The dicarboxylic acids containing no mercaptan group (i) which may be used are generally of the formula HOOC-R<sup>2</sup>-COOH, where R<sup>2</sup> represents a divalent

aliphatic, aromatic, or alicyclic residue, and include succinic, adipic, phthalic, hexahydrophthalic, sebacic, and malic acids, and dimerised fatty acids or their anhydrides. Although they can be used, ethylenically-unsaturated dicarboxylic acids are not preferred.

The dicarboxylic acids (m) and their anhydrides may be selected from those listed above for (i) and also the mercaptan-containing dicarboxylic acids (g) and their anhydrides.

It is often desirable, when preparing a polymercaptan ester for use in the present invention to incorporate a monofunctional compound such as a monocarboxylic acid (j) or a monohydric alcohol (k) as a chain-terminator. Examples of these are aliphatic alcohols such as methanol, ethanol, 2-ethylhexanol, 2-methoxyethanol, and monoethyl ethers of poly(oxethylene) glycols and poly(oxypropylene) glycols; cycloaliphatic alcohols such as cyclohexanol; aliphatic carboxylic acids such as acetic acid, 2-ethylhexanoic acid, stearic acid, and oleic acid; and aromatic acids such as benzoic acid. As already indicated, it is especially advantageous to use as the chain-terminator a compound which contains a mercaptan group, examples being monomercaptomonocarboxylic acids and monomercaptomonohydric alcohols and, more specifically, thioglycollic acid, 2-mercaptopropionic acid, 3-mercaptopropionic acid, 2-mercaptopropano, and 2-mercaptopropan-1-ol.

The polymercaptan esters are, in general, known substances (see U.S. Pat. Nos. 2,456,314, 2,461,920, 2,914,585, and 3,138,573, French Patent Specification No. 1503633 and British Specification No. 941829).

The preferred polymercaptan esters used in the process of the present invention contain, directly attached to carbon atoms, an average n groups of formula



where

a and b are each zero or 1 but are not the same, n is an integer of at least 1 and at most 6,

Y and Z each represent a divalent organic radical, and

X represents a divalent organic radical which must contain an —SH group when n is 1.

More specifically, the average structures of the preferred esters can be represented by one of the formulae



and especially by one of the formulae





where

$\text{R}^2$  denotes the residue of an aliphatic, cycloaliphatic, or aromatic dicarboxylic acid after removal of the two carboxyl groups,

$\text{R}^3$  denotes the residue of an aliphatic, araliphatic, or cycloaliphatic diol after removal of the two hydroxyl groups,

$\text{R}^4$  denotes an organic radical containing at least two carbon atoms and directly linked through carbon atoms thereof to the indicated mercaptan-terminated ester chains,

$\text{R}^5$  denotes the residue of an aliphatic, cycloaliphatic, or aromatic dicarboxylic acid containing a mercaptan group, after removal of the two carboxyl groups,

$m$  is an integer of at least 1,

$p$  is an integer of at least 2, and

$\text{R}$ ,  $\text{r}$ , and  $t$  have the meanings previously assigned.

It will be understood that formulae II to XVII represent the average structure of the esters. Because of incomplete esterification, other substances may also be present. Further, as already indicated, not all units designated  $\text{R}$ ,  $\text{R}'$ , and  $\text{R}^2$  to  $\text{R}^5$  need be the same.

Many of the esters are insoluble in water but can be applied as aqueous dispersions or emulsions. They may also be applied from organic solvents, for example lower alkanols (such as ethyl alcohol), lower ketones (such as ethyl methyl ketone), xylene, and halogenated hydrocarbon solvents, especially chlorinated and/or fluorinated hydrocarbons containing not more than three carbon atoms such as the dry cleaning solvents, carbon tetrachloride, trichloroethylene, and perchloroethylene.

The amount of the ester to be used depends on the effect desired. For most purposes a pick-up of from 0.1 to 1 percent, and at most 10 percent, by weight based on the material to be treated is preferred. The "handle" of the treated material will, of course, depend on the amount of ester employed and by simple experiment the least amount required to give the desired effect may readily be determined. Further, the composition and the construction of the fabrics, also influence the amount of ester required.

If desired, the ester may be used in conjunction with other agents which can be made to cross-link on the fibres, e.g., aminoplasts and polyepoxides.

The desired effects may not be fully obtainable until substantially all the ester has cured. At room temperatures (say, 20°C) this may take from five to ten days or even longer, but occurs much more rapidly at higher temperatures. The curing reaction may also be accelerated greatly by a catalyst and generally it is preferred to add the catalyst to the material to be treated at the same time as the ester is applied although it may be added before or afterwards if desired. The curing time can be controlled by selecting an appropriate catalyst and the choice of curing time will depend on the particular application of the process according to the invention. The catalysts may be bases, siccatives, oxidative curing agents, sulphur, sulphur-containing organic compounds, salts and chelates of heavy metals, and free-radical catalysts or combination of these.

As organic bases there may be used primary or sec-

### XVII

ondary amines such as the lower alkanolamines, e.g., mono- and di-ethanolamine, and polyamines, e.g., ethylenediamine, diethylenetriamine, triethylenetetramine, tetraethylenepentamine, and hexamethylenediamine. As inorganic bases there may be used the water-soluble oxides and hydroxides, e.g., sodium hydroxide, water-soluble strongly basic salts such as trisodium phosphate, disodium tetraborate, and sodium carbonate, and also ammonia.

As sulphur-containing organic compounds there may be used compounds in which the sulphur atoms are not exclusively present as mercaptan groups and which are mercaptobenzothiazoles and their derivatives, dithiocarbamates, thiuram sulphides, thiorea, disulphides, alkyl xanthogen sulphides and alkyl xanthates.

Examples of siccatives are calcium, copper, iron, lead, cerium, and cobalt naphthenates.

Examples of suitable free-radical catalysts are azodisobutyronitrile and various peroxides and hydroperoxides such as hydrogen peroxide, cumene hydroperoxide, tert-butyl hydroperoxide, dicumyl peroxide, dilauryl peroxide, methyl ethyl ketone peroxide, diisopropyl peroxydicarbonate, and chlorobenzoyl peroxide. Particularly convenient to use are aqueous solutions of hydrogen peroxide.

Yet other catalysts are salts of a heavy metal with an acid having an acid strength ( $-\log pK$ ) below 5, or chelates of a heavy metal, including chelates which are also salts. By "heavy metal" is meant one classified as "heavy" in Lange's Handbook of Chemistry, revised 10<sup>th</sup> Edition, McGraw-Hill Book Co., at pp. 60-61, that is, a metal of group IB, IIB, IIIB, IVB, VB, VIB, VIIB, or VIII, a metal of group IIIA having an atomic number of at least 13, a metal of group IVA having an atomic number of at least 51. Preferably the metal is a member of Group IB, IIB, IVB, VB, VIB, VIIB, or VIII, particularly the first series of such metals, i.e., titanium, vanadium, chromium, manganese, nickel and especially iron, cobalt, and copper. Suitable salt-forming, non-drying acids are mineral acids, especially hydrochloric, hydrobromic, nitric, sulphuric, phosphorous, and phosphoric acids, and organic acids such as chloroacetic, fumaric, maleic, oxalic, salicylic and, more especially, citric acid. Suitable chelating agents include those in which the chelating atoms are oxygen and/or nitrogen, for example, 1,2- and 1,3-diketones such as acetylacetone, alkylenediamines such as ethylenediamine, and more particularly ethylenediaminetetra-acetic acid.

The amount of catalyst used can vary widely. In general from 0.1 to 20 percent, and preferably 1 to 10 percent, by weight based on the weight of the ester used is required, although much larger quantities can be used. Curing of the ester takes place more rapidly at a pH of more than 7, e.g., from 7.5 to 12.

As indicated above, curing of the ester is also assisted by using elevated temperatures, e.g., from 30° to as high as 180°C, but temperatures of more than 180°C, say, up to 220°C, may be encountered if curing is combined with heat-setting. In high humidities also, curing is accelerated.

The ester and the catalyst if used, can be applied to the material in conventional ways. For example, where fabric or yarn is to be treated, they may be padded on from a solution, emulsion, or suspension, or the mate-

rial may be immersed in a bath. If garments or garment pieces are to be treated then it is convenient to spray them or to tumble them with the solution, emulsion, or suspension.

A particularly effective way of carrying out the process of this invention involves applying the ester by an exhaustion process and comprises immersing the fibres in an aqueous medium containing the ester and heated at from 25° to 95°. Exhaustion is favoured by working under acid conditions, the aqueous medium having a pH of from 3 to 6. 5 10

It is particularly convenient to use an aqueous emulsion comprising:

- i. an ester as aforesaid
  - ii. an emulsifying agent which is preferably nonionic or anionic (for example, compounds containing polyoxyethylene chains),
  - iii. a protective colloid (such as sodium carboxymethylcellulose, hydroxyethylcellulose and methoxyethylcellulose, and a methyl vinyl ether-maleic anhydride copolymer in the form of an alkali metal or ammonium salt).

The compositions used in the process of this invention may contain bacteriostatic, rotproofing, flame-proofing, or wetting agents, and other antisoiling and antistatic agents. They may also contain water-repellents, such as paraffin wax, and fluorescent whitening agents.

The following Examples illustrate the invention. Unless otherwise specified, parts and percentages are by weight. The esters used were prepared as follows. 30

### Thiol A

A mixture of "Trimer acid Empol 1043" (87.6 g), polyoxypropylene glycol of average molecular weight 425 (127.5 g), thioglycollic acid (27.6 g), toluene-p-sulphonic acid (2g), and perchloroethylene (300 ml) was heated under reflux in an atmosphere of nitrogen. Water formed during the reaction (11 ml) was removed as its azeotrope with perchloroethylene. The mixture was cooled, and washed with water, the organic layer was separated, and the solvent was evaporated off to leave Thiol A (226.4 g) having a thiol content of 1.09 equiv./kg.

Other thiol esters which were prepared in a similar manner are listed in Table I, except that, in making Thiol N, the toluene-p-sulphonic acid was replaced by 1 ml of 50 percent aqueous sulphuric acid.

TABLE I-Continued

| Thiol | Substance                                        | Components | Molar ratio | Thiol content (equiv./kg) |
|-------|--------------------------------------------------|------------|-------------|---------------------------|
| G     | thioglycollic acid                               | 3          |             |                           |
|       | hexane-1,2,6-triol                               | 1          |             | 0.94                      |
|       | "Dimer acid Empol 1022"                          | 5          |             |                           |
|       | hexane-1,6-diol                                  | 4          |             |                           |
|       | thioglycollic acid                               | 2.5        |             |                           |
| H     | "Trimer acid Empol 1043"                         | 1          |             | 1.64                      |
|       | butane-1,4-diol                                  | 3          |             |                           |
|       | thioglycollic acid                               | 3          |             |                           |
| I     | polyoxypropylene triol,<br>average mol.wt.700    | 1          |             | 1.78                      |
| J     | adipic acid                                      | 3          |             |                           |
|       | butane-1,4-diol                                  | 3          |             |                           |
|       | thioglycollic acid                               | 3          |             |                           |
|       | hexane-1,2,6-triol                               | 1          |             | 0.99                      |
| K     | "Dimer acid Empol 1022"                          | 2          |             |                           |
|       | polyoxypropylene glycol,<br>average mol.wt.425   | 2          |             |                           |
|       | thioglycollic acid                               | 3          |             |                           |
|       | glycerol                                         | 1          |             | 2.07                      |
| L     | adipic acid                                      | 2          |             |                           |
|       | polyoxyethylene glycol,<br>average mol.wt.400    | 2          |             |                           |
|       | thioglycollic acid                               | 3          |             |                           |
| M     | 1,1,1-trimethylolpropane                         | 1          |             | 0.82                      |
|       | succinic acid                                    | 4          |             |                           |
|       | "Comerginol 65"                                  | 4          |             |                           |
| N     | thioglycollic acid                               | 3          |             |                           |
|       | "Trimer acid Empol 1043"                         | 1          |             | 2.11                      |
|       | butane-1,4-diol                                  | 3          |             |                           |
| O     | 3-mercaptopropionic acid                         | 3          |             |                           |
|       | 1,1,1-trimethylolpropane                         | 1          |             | 1.63                      |
|       | adipic acid                                      | 2          |             |                           |
| P     | 2,2-bis(p-(2-hydroxypropoxy)<br>phenyl) propane  | 2          |             |                           |
|       | thioglycollic acid                               | 3          |             |                           |
|       | glycerol                                         | 1          |             | 1.10                      |
| Q     | adipic acid                                      | 4          |             |                           |
|       | polyoxypropylene glycol,<br>average mol.wt.425   | 4          |             |                           |
|       | thioglycollic acid                               | 3          |             |                           |
| R     | polyoxypropylene triol,<br>average mol.wt.700    | 1          |             | 1.36                      |
|       | adipic acid                                      | 3          |             |                           |
|       | 2,2-bis(p-(2-hydroxypropoxy)<br>phenyl) propane  | 3          |             |                           |
| S     | thioglycollic acid                               | 3          |             |                           |
|       | "Trimer acid Empol 1043"                         | 1          |             | 0.85                      |
|       | polyoxyethylene glycol,<br>average mol.wt.300    | 3          |             |                           |
| T     | thioglycollic acid                               | 3          |             |                           |
|       | polyoxypropylene triol,<br>average mol.wt.3000   | 1          |             | 0.48                      |
|       | succinic anhydride                               | 3          |             |                           |
| U     | 2-mercaptopropanol                               | 3          |             |                           |
|       | pentaerythritol-propylene<br>oxide tetrol adduct | 1          |             |                           |
|       | average mol.wt.650                               |            |             |                           |
| V     | "Dimer acid Empol 1022"                          | 4          |             |                           |
|       | 2-mercaptopropanol                               | 4          |             |                           |
|       | glycerol                                         | 1          |             |                           |
| W     | phthalic anhydride                               | 4          |             |                           |
|       | butane-1,4-diol                                  | 4          |             |                           |
|       | thioglycollic acid                               | 3          |             |                           |
| X     | polyoxypropylene glycol<br>average mol.wt.1000   | 6          |             | 0.58                      |
|       | mercaptosuccinic acid                            | 5          |             |                           |
| Y     | polyoxypropylene glycol<br>average mol.wt.2000   | 11         |             | 0.40                      |
|       | mercaptosuccinic acid                            | 10         |             |                           |
| Z     | polyoxypropylene glycol<br>average mol.wt.425    | 11         |             | 1.65                      |
|       | mercaptosuccinic acid                            | 10         |             |                           |
| A'    | butane-1,4-diol                                  | 6          |             | 3.98                      |
|       | mercaptosuccinic acid                            | 5          |             |                           |
|       | "Comerginol 65"                                  | 2          |             | 1.79                      |
| A'    | mercaptosuccinic acid                            | 1          |             |                           |
|       | thioglycollic acid                               | 2          |             |                           |
|       | polyoxypropylene glycol<br>average mol.wt.425    | 11         |             | 0.93                      |
| A'    | mercaptosuccinic acid                            | 6          |             |                           |
|       | adipic acid                                      | 4          |             |                           |
| A'    | acetic acid                                      | 2          |             |                           |

"Trimer acid Empol 1043" is available from Unilever-Emery N.V., Gouda, Holland. It is a trimerised unsaturated C<sub>18</sub> fatty acid, having an average molecular weight of about 800 and a carboxyl content of about 3.4 equiv./kg. "Dimer acid Empol 1022" was obtained from the same source: it is a dimerised unsaturated C<sub>18</sub> fatty acid, having an average molecular weight of about 570 and a carboxyl content of about 3.4 equiv./kg. "Comerginol 65" was obtained from Bibby Chemicals Ltd., Liverpool. It has an average molecular weight of about 700, and a hydroxyl value of 155-165. It consists essentially of diprimary alcohols, prepared by catalytic hydrogenation of the methyl esters of long chain aromatic-aliphatic fatty acids, together with, as by-products, small amounts of monohydric and trihydric alcohols.

#### EXAMPLE 1

Samples of "Crimplene" (Registered Trade Mark) scoured polyester fabric were padded with a 1 percent solution of Thiols A, B, C, or D in trichloroethylene to 125 percent uptake. The samples were dried in an oven at 60°C for 30 minutes and then allowed to stand overnight at room temperature. All samples had a softer handle than had untreated "Crimplene".

#### EXAMPLE 2

Aqueous emulsions were prepared containing:

|                               |       |
|-------------------------------|-------|
| Thiol                         | 500 g |
| Emulsifying agent             | 50 g  |
| Sodium carboxymethylcellulose | 5 g   |
| Water                         | 445 g |

The components were mixed at room temperature with a Silverson mixer until uniform emulsion resulted. The emulsifying agent was an adduct of a mixture of C<sub>16</sub> and C<sub>18</sub> aliphatic primary amines (1 mol.) with ethylene oxide (70 mol.).

Emulsions containing Thiols C and D were applied at 2 percent on weight of fabric on samples of scoured "Crimplene" at 60°C using a liquor ratio of 20:1. The pH of the baths was adjusted to 3.5 with acetic acid to accelerate the exhaustion of the ester onto the fibre. After 15 minutes hydrogen peroxide was added until the concentration of hydrogen peroxide in the bath was 0.3 percent. During the treatment, the solutions, which were originally cloudy, became progressively clearer, showing that the resin emulsion was exhausting onto the fabric.

After a total of 30 minutes the baths were clear and the samples were removed, spun in a spin-drier, and dried in an oven at 60°C for 30 minutes. After they had been left overnight at room temperature they were found to have a better handle, compared to untreated samples. This excellent handle was retained when the "Crimplene" was washed in a solution of 1 g/l surfactant for 10 minutes at 55°C. (The surfactant was an adduct of 1 mol. of nonylphenol with 9 mol. of ethylene oxide).

#### EXAMPLE 3

Hanks of yarns made of nylon, "Courtelle" and "Acrilan" (polyacrylonitriles), and "Tricel" (cellulose tri-

acetate) were treated with the emulsions described in Example 2 by the following procedure. The yarns were immersed in the emulsion at 60°C adjusted to pH 4.0 with 0.3 g/l acetic acid using a liquor ratio of 20:1. After being treated for 30 minutes the yarns were spun in a spin-drier, dried in an oven at 70°C, and finally air-conditioned. The handle of the yarns was then assessed.

The nylon and "Acrilan" yarns had a pleasing softer handle. Although the effect on the "Tricel" and "Courtelle" yarns was not quite as outstanding as on the nylon and "Acrilan", nevertheless, an appreciably softer handle was obtained.

The words "Courtelle", "Acrilan", and "Tricel" are Registered Trade Marks.

#### EXAMPLE 4

Polyester plain weave fabric was padded with trichloroethylene solutions of Thiols D and E with and without diethylenetriamine. The uptake of Thiol was 2 percent and of diethylenetriamine, if present, 0.04 percent. The patterns were dried for 10 minutes at 60°C and they, and a piece of untreated material were heat-set at 195°C for 30 seconds. Compared with untreated fabric, all the treated materials had a softer handle and far superior antistatic properties. (The antistatic test consisted of placing the fabric samples about 1 cm above a tray of cigarette ash: untreated material was completely covered with ash whereas there was no pick-up of ash by the treated material). Similar results were obtainable using trichloroethylene solutions of Thiols G - Q.

#### EXAMPLE 5

Samples of scoured 'Crimplene' were padded to 185 percent pick-up with Emulsions 1 - 18. These emulsions were prepared in the same manner as described in Example 2. The treated patterns were dried for 30 minutes at 80°C. The antistatic properties of the treated fabric were assessed by rubbing the fabrics on a wooden surface and then placing them about 1 cm above a bowl of sawdust and noting the amount of sawdust picked up by the fabric.

Antisoil-redeposition and soil-release properties of treated and untreated samples were measured by the following method. Each pattern was screen printed in a striped pattern with three different soiling compositions, each applied as a band 3 cm wide and separated from the adjoining band by an unsoiled strip of the same width.

Soil A was a mixture of used, dirty motor oil (50 percent) and petroleum jelly (50 percent)

Soil B was a mixture of lanolin (84 percent and trichloroethylene (16 percent)

Soil C was a mixture of sieved vacuum cleaner dust (20 percent), lanolin (60 percent) and trichloroethylene (20 percent).

The soiled patterns were dried in an oven for 1 hour at 40°C. Portions of the treated and untreated soiled patterns were then washed for 30 minutes in a washing machine at 40°C in a solution containing 2.5 g/l of an anionic detergent. After being well rinsed with water, the patterns were finally dried at 50°C for 1 hour, and the soil release and antisoil-redeposition properties were noted.

TABLE II

| Emulsion  | % Agent       | % Catalyst              | Antistatic effect | Soil-release effect | Antisoil redeposition effect |
|-----------|---------------|-------------------------|-------------------|---------------------|------------------------------|
| 1         | 2% Thiol A    | —                       | Good              | V. Good             | V. Good                      |
| 2         | 2% Thiol A    | 0.2% NaHCO <sub>3</sub> | Good              | V. Good             | V. Good                      |
| 3         | 2% Thiol B    | —                       | Good              | Good                | V. Good                      |
| 4         | 2% Thiol B    | 0.2% NaHCO <sub>3</sub> | Good              | Good                | V. Good                      |
| 5         | 2% Thiol C    | —                       | Good              | Good                | V. Good                      |
| 6         | 2% Thiol C    | 0.2% NaHCO <sub>3</sub> | Good              | Good                | V. Good                      |
| 7         | 2% Thiol C    | 0.2% SBUD*              | V. Good           | Good                | V. Good                      |
| 8         | 2% Thiol C    | 0.2% CuSO <sub>4</sub>  | Bad               | Good                | V. Good                      |
| 9         | 2% Thiol C    | 0.2% MEA*               | Good              | V. Good             | V. Good                      |
| 10        | 2% Thiol D    | —                       | Good              | Good                | V. Good                      |
| 11        | 2% Thiol D    | 0.2% NaHCO <sub>3</sub> | V. Good           | Good                | V. Good                      |
| 12        | 2% Thiol E    | —                       | Good              | F. Good             | Good                         |
| 13        | 2% Thiol E    | 0.2% NaHCO <sub>3</sub> | Good              | F. Good             | Good                         |
| 14        | 2% Thiol F    | —                       | Good              | V. Good             | V. Good                      |
| 15        | 2% Thiol F    | 0.2% NaHCO <sub>3</sub> | Good              | V. Good             | V. Good                      |
| 16        | 2% Polyol A   | 0.2% NaHCO <sub>3</sub> | Good              | Bad                 | Bad                          |
| 17        | 2% Softener 1 | —                       | F. Good           | Bad                 | V. Bad                       |
| 18        | 2% Softener 2 | —                       | Good              | Bad                 | V. Bad                       |
| Untreated |               |                         | Bad               | V. Bad              | V. Bad                       |

\* SBUD = sodium dibutylthiocarbamate

MEA = monoethanolamine

V. Good = very good

F. Good = fairly good

V. Bad = very bad

'Softener 1' was a commercially available cationic softening agent prepared from a long chain fatty acid, a

polyamine, and an unsaturated nitrile.

'Softener 2' was a commercially available polyethylene emulsion.

'Polyol A' was a polyoxypropylene triol of molecular weight 4000.

Similar results were obtainable using emulsions of 40  
Thiols R - Z and A'.

We claim:

1. A process for improving the handle of synthetic  
fibres which comprises the steps of

1. applying to the fibres, in the absence of keratinous 45  
material, a dispersion of a thiol-containing poly-  
ester material in water or organic solvent, and

2. curing the polyester material on the fibres, wherein  
the polyester material has an average molecular  
weight of between 400 and 10,000 and is of the for- 50  
mulae:



and



where

R<sup>2</sup> denotes the residue of an acid of 4 to 36 carbon  
atoms selected from aliphatic, cycloaliphatic, and  
aromatic dicarboxylic acids after removal of the  
two carboxylic groups,

R<sup>3</sup> denotes the residue of a diol of at least 4 carbon  
atoms selected from aliphatic, araliphatic, and cy-  
cloaliphatic diols after removal of the two hydroxyl  
groups,

R<sup>4</sup> denotes an organic radical containing at least 2  
carbon atoms and directly linked through carbon  
atoms thereof to the indicated mercaptan-  
terminated ester chains.

R<sup>5</sup> denotes the residue of an acid of three to four car-  
bon atoms selected from aliphatic, dicarboxylic  
acids containing a mercaptan group, after removal  
of the two carboxyl groups,

m is an integer of at least 1,

p is an integer of at least 2 and no more than 6 and  
R is a divalent hydrocarbon radical of 1 to 24 carbon  
atoms.

2. Process according to claim 1, in which there is  
used from 0.1 to 10 percent by weight of the polyester  
material, calculated on the weight of the synthetic  
fibres treated.

3. Process according to claim 1 in which the synthetic  
fibres are selected from the group consisting of nylons,  
polyesters, polyacrylonitriles, polyvinyl alcohols, and  
cellulose triacetate.

4. Process according to claim 1, wherein the poly-  
ester material is applied to the fibres by an exhaustion  
process comprising immersing them in an aqueous me-  
dium which contains the ester and which is heated to  
a temperature in the range 25° to 95°C.

5. Process according to claim 1 wherein the polyester material is applied to the fibres in an aqueous medium having a pH of from 3 to 6.

6. Process according to claim 1, wherein a catalyst for curing the polyester material is also applied which is selected from the group consisting of bases, siccatives, oxidising agents, sulfur, sulfur-containing organic compounds, free-radical catalysts, salts of a heavy metal with an acid having an acid strength ( $-\log pK$ ) below 5, and chelates of a heavy metal, including chelates which are also salts.

7. Process according to claim 1, in which the curing of the polyester material is effected at a temperature in the range 30° to 180°C.

8. Process according to claim 1, in which the curing of the polyester material is effected at a pH in the range 7.5 to 12.

9. The process of claim 1, wherein the polyester material is selected from the formulae:  
 I, IV, and V where R is  $-C_6H_{2t}-$   
 II, III, IV, and VIII where R is  $-C_rH_{2r}-$ ; and  
 VII and VIII where R<sup>5</sup> is



wherein r is an integer of 1 to 24, t is an integer of 2 to 18, and the average molecular weight of the polyester material is 400 to 10,000.

10. Synthetic fibrous material, free from keratinous material, bearing thereon an polyester material as specified in claim 1.

\* \* \* \* \*

20

25

30

35

40

45

50

55

60

65